

# UNITED STATES PATENT OFFICE.

JOHN V. WICKS, OF SEATTLE, WASHINGTON, ASSIGNOR TO MARVEL MANUFACTURING CO., OF SEATTLE, WASHINGTON, A FIRM COMPOSED OF W. D. TRIPPLE, GEORGE TRIPPLE, AND J. V. WICKS.

## VALVE-GRINDING COMPOUND.

1,381,953.

Specification of Letters Patent. Patented June 21, 1921.

No. Drawing.

Application filed June 3, 1920. Serial No. 386,327.

To all whom it may concern:

Be it known that I, JOHN V. WICKS, a citizen of the United States, and resident of Seattle, in the county of King and State 5 of Washington, have invented certain new and useful Improvements in Valve-Grinding Compounds, of which the following is a specification.

My invention consists of an improvement 10 in compounds for grinding valves, such, for instance, as the valves of an internal combustion engine.

It is essential, in this work, that the compound be of such character that small particles 15 will not fall from the valve seat, while in use or while being made ready for grinding, and in this manner enter the cylinder. It is an object of my invention to form a compound which will be of such a character 20 and consistency, under all conditions, that it will not permit particles to be separated from the mass, but which will permit the abrasive to work freely and quickly upon the valve seat.

Another object of my invention is to produce a valve grinding compound which will 25 cut rapidly, without scoring or forming rings in the valve or its seat.

Another object of my invention is to form 30 a superior valve grinding compound which may be sold ready-mixed, and which will require the addition of no other ingredients in use.

The compound which is my invention will 35 be hereinafter described in this specification, and those materials and combinations thereof, and the proportions which I consider preferable, will be particularly set forth in the appended claims.

As the base for my compound I employ 40 a non-fluid oil. This oil, which forms the vehicle for the other elements, should be such that it will not become fluid under ordinary temperatures, nor under the temperatures 45 attained during the action of grinding. For such purposes I have found petroleum hard oil to be suitable.

With this hard oil I mix a powdered or pulverized abrasive, such as carborundum, 50 which will abrade the very hard valve seats.

For varying conditions of work, and for variations in the speed of cutting and smoothness of finish desired, various grades 55 of abrasive may be used. I have employed carborundum varying from No. F1 to 180 grade, although it is obvious that for a finer finish a finer grade of abrasive than No. F1 might be employed, or for a rougher 60 finish, a coarser grade than 180 might be employed.

The third ingredient which I employ is known as lard oil. This oil appears to assist materially in the abrasive action, 65 although the principle of its action is not understood. It may be that this oil prevents the formation of a film between the grinding surfaces, and it may assist in removing the minute particles which are 70 ground away. Other similar oils might be employed, but I have found that the best results are secured when lard oil is employed.

The three ingredients named, or their 75 equivalents, are thoroughly intermixed, and the product is a paste which is ready for use, without the addition of other substances. The proportions may be varied to suit the purpose for which the compound is to be 80 used, but in general I have found that the best results are secured, in valve grinding, when the substances named are mixed in equal proportions by weight. I do not desire to limit myself to this exact proportion, 85 however, as it is evident that if a rougher job were desired, the proportion of carborundum might be increased, or if the work were to be performed at high speeds, the proportion of petroleum hard oil might be 90 increased, as this oil acts as the binder or homogenizer, to keep the mixture together without becoming fluid. If it is desired to produce a very smooth finish, the proportion of lard oil might be increased. Other 95 considerations might make it desirable to increase the proportion of any two of the ingredients with respect to the other.

Although my compound is particularly designed for and peculiarly adapted for 100 valve grinding, it may be used for any purpose for which it is found suitable, or in

any place where it is desired to produce a smooth surface with very little effort and quickly. I do not desire to be understood as limiting the use of my grinding compound to the sole use of grinding valves.

5 What I claim as my invention is:—

1. A valve grinding compound comprising a non-fluid oleaginous vehicle, an abrasive and lard oil intermixed therewith.

10 2. A valve grinding compound compris-

ing petroleum hard oil, a pulverized abrasive, and lard oil, intermixed.

3. A valve grinding compound comprising substantially equal parts by weight of petroleum hard oil, carborundum, and lard oil, intermixed.

Signed at Seattle, Washington, this 28th day of May, 1920.

JOHN V. WICKS.